

## 1

2,993,862

ACETYLENIC GLYCOLS AS CORROSION  
INHIBITORS

Roger F. Monroe and Fred J. Lowes, Midland, Mich., and Gerald L. Foster and Billy D. Oakes, Tulsa, Okla., assignors to The Dow Chemical Company, Midland, Mich., a corporation of Delaware  
No Drawing. Filed Aug. 2, 1956, Ser. No. 601,641  
6 Claims. (Cl. 252—146)

This invention relates to corrosion inhibitors for use in aqueous hydrochloric acid to inhibit the corrosion of iron, steel, nickel or ferrous alloy metals exposed to said aqueous acid.

We have now discovered that certain acetylenic glycols, specifically, those having the formula



wherein R is a radical selected from the group consisting of —H and —CH<sub>3</sub> are potent corrosion inhibitors and, as such, are particularly effective in protecting iron, steel, ferrous alloys and nickel from the corrosive attack of aqueous hydrochloric acid. By the term "aqueous hydrochloric acid" we mean HCl in the presence of a significant amount of water and do not mean to exclude the presence of other substances.

According to the invention, the inhibitors are simply dissolved in the hydrochloric acid solution the corrosive action of which is to be inhibited. Only a small amount of inhibitor is required. As little as a few thousandths of 1 percent, based on the acid solution, significantly reduces the corrosion of iron and nickel exposed to the acid. The degree of inhibition increases with the concentration of the inhibitor up to a concentration of about 1 percent. Beyond this point there is little advantage in using more inhibitor.

The inhibitors of the invention are effective not only at ordinary temperatures but also at elevated temperatures, up to the point at which the inhibitors decompose. They are effective in all concentrations of hydrochloric acid up to and including commercial concentrated acid (about 36 percent). Applications in which they are particularly useful include metal-cleaning baths, oil well-treating acids, boiler-cleaning solutions and the like.

In order to illustrate the effectiveness of our corrosion inhibitors we have conducted tests in which hydrochloric acid at various concentrations and containing 0.4 percent of the inhibitor being tested is placed in contact with a standard coupon of the metal to be protected. After 16 hr. the coupon is washed, dried and weighed to determine the amount of metal dissolved by the acid. From this is calculated the corrosion rate in terms of inches of penetration per year. Some typical results thus obtained are shown in Table I.

TABLE I

Corrosion rates, inches penetration per year, of steel and nickel exposed to hydrochloric acid

|                              | Inhibitor (0.4 percent) |                                     |                        |
|------------------------------|-------------------------|-------------------------------------|------------------------|
|                              | None                    | 2,7-Dimethyl-3,5-octadiyne-2,7-Diol | 2,4-Hexadiyne-1,6-Diol |
| 10% HCl, 150° F.: Mild Steel | >10                     | 0.074                               | 0.108                  |
| 36% HCl, 25° F.: Mild Steel  | 0.40                    | 0.24                                |                        |
| Nickel                       | .26                     | .07                                 |                        |
| 5% HCl, 25° F.: Nickel       |                         | .01                                 |                        |

Results similar to those shown in Table I were ob-

## 2

tained when other concentrations of hydrochloric acid, other temperatures in the range from room temperatures up to the decomposition point of the inhibitor, and other ferrous metals were used instead of those used in obtaining the data in Table I. It was also found that the effectiveness of the inhibitors was not impaired by the presence of liquids other than water, such as, for instance, alcohols, glycols or surfactants. Likewise, their effectiveness was not impaired by the presence of various salts in the aqueous acid such as the soluble chlorides and sulfates.

We claim:

1. Aqueous hydrochloric acid containing about 5 to 36% concentration, by weight, and, as the sole active corrosion inhibitor therefor an effective amount of a compound having the formula



wherein R is a radical selected from the group consisting of —H and —CH<sub>3</sub>.

2. A solution as in claim 1 wherein R is —H.

3. A solution as in claim 1 wherein R is —CH<sub>3</sub>.

25 4. A solution as in claim 1 wherein the concentration of the inhibitor is from a few thousandths percent to about one percent, by weight.

5. A process for inhibiting the corrosion of a metal of the group consisting of iron, steel, nickel and ferrous alloys by aqueous hydrochloric acid in contact therewith comprising maintaining in said acid a small but effective concentration of the inhibitor having the formula



35 wherein R is a radical selected from the group consisting of —H and —CH<sub>3</sub>.

6. A process as defined in claim 5 wherein the concentration of inhibitor is from a few thousandths percent to about 1 percent, by weight.

## References Cited in the file of this patent

## UNITED STATES PATENTS

|           |                     |                |
|-----------|---------------------|----------------|
| 1,169,341 | Chrzesciuski et al. | Jan. 25, 1916  |
| 1,841,768 | Straus et al.       | Jan. 19, 1932  |
| 1,963,934 | Carothers et al.    | June 19, 1934  |
| 2,152,406 | Ducamp et al.       | Mar. 28, 1939  |
| 2,204,597 | Humphreys et al.    | June 18, 1940  |
| 2,250,445 | Bruson et al.       | July 29, 1941  |
| 2,355,599 | Walker              | Aug. 8, 1944   |
| 2,371,644 | Petering et al.     | Mar. 20, 1945  |
| 2,407,149 | Gardenier           | Sept. 3, 1946  |
| 2,603,622 | Berger et al.       | July 15, 1952  |
| 2,726,269 | Humphlett           | Dec. 6, 1955   |
| 2,775,624 | Skeeters et al.     | Dec. 25, 1956  |
| 2,775,626 | Schaaf et al.       | Dec. 25, 1956  |
| 2,805,257 | Lowes et al.        | Sept. 3, 1957  |
| 2,806,067 | Monroe et al.       | Sept. 10, 1957 |
| 2,814,593 | Beiswanger et al.   | Nov. 26, 1957  |
| 2,838,458 | Bachtel             | June 10, 1958  |
| 2,880,180 | Foster et al.       | Mar. 31, 1959  |

## FOREIGN PATENTS

|               |           |                |
|---------------|-----------|----------------|
| Great Britain | 627,453   | Aug. 9, 1949   |
| Germany       | 890,796   | Sept. 21, 1953 |
| Belgium       | 505,421   | Sept. 15, 1951 |
| France        | 1,075,385 | Apr. 14, 1954  |
| France        | 1,079,916 | May 26, 1954   |

## OTHER REFERENCES

70 Corrosion Handbook by Uhlig, pp. 910-912, pub. by John Wiley, N.Y., 1948.